

1

2,797,162

## LOW ALLOY STEEL FOR SUB-ZERO TEMPERATURE APPLICATION

Michael Korczynsky, Niagara Falls, N. Y., assignor to Union Carbide and Carbon Corporation, a corporation of New York

No Drawing. Application July 19, 1954,  
Serial No. 444,378

8 Claims. (Cl. 75—124)

This invention relates to low alloy steel for use at low temperature, and more particularly to alloys suitable for use in applications where superior impact resistance at sub-zero temperatures is required.

The trend of modern engineering practice is toward the utilization of extremely low temperatures for many and diverse operations. Steels with properties which permit their efficient use at sub-zero temperatures are needed for chemical apparatus, piping, pressure vessels and for facilities for the storage and transportation of liquid gases.

The low temperature failures of steel articles usually result from low notched bar impact strength, so that the notch sensitivity of these materials is the critical factor in their selection. In general, materials having an impact value of at least 15 foot pounds at a given temperature as determined by Charpy key hole impact tests are likely to have adequate toughness for application at a similar service temperature.

Several alloys have been proposed for use at low temperatures, but the utility of each one of them has been limited for various reasons. Of these, austenitic and high alloy ferritic steels have the disadvantage of being quite costly, of being difficult to fabricate, and of requiring critical heat treating conditions for optimum properties. Economical low alloy steels do not retain their toughness to sufficiently low temperatures. In the case of these alloys, variation in the heat treatment, because of its criticality, will alter its properties, thereby rendering difficult the reproducibility of the desired properties of the steel. Hitherto, austenitic stainless steel has been the most efficient steel for low temperature service, but its wide applicability has been limited by economic factors.

of alloys whose heat treatment is not critical. A more specific object is the provision of low alloy steel articles having a mean value of toughness in excess of 15 foot pounds in the Charpy key hole impact tests at temperatures as low as about —196° C.

The invention by means of which these objects are achieved is based on the discovery that the addition of small properly proportioned quantities of tantalum and optionally columbium to chromium-copper-nickel steels, 10 produces a remarkable lowering of the transition temperatures of such alloys.

This invention comprises alloys containing 0.02% to 0.15% carbon, 0.20% to 1.20% manganese, 0.05% to 0.60% silicon, 0.20% to 1.20% copper, 0.25% to 1.50% chromium, 1.0% to 5.0% nickel, 0.03% to 0.30% aluminum, up to 0.025% nitrogen and 0.05% to 0.25% in the aggregate of tantalum and columbium, the tantalum content being at least 0.04%, the remainder of the alloys being iron, except for incidental impurities and small quantities of elements customarily found in steels of good quality. The preferred range of percentages for the alloys of this invention is as follows:

|           | Percent    |
|-----------|------------|
| Carbon    | 0.02-0.10  |
| Manganese | 0.20-0.60  |
| Silicon   | 0.10-0.35  |
| Copper    | 0.20-0.60  |
| Chromium  | 0.50-0.90  |
| Nickel    | 2.00-3.00  |
| Aluminum  | 0.05-0.20  |
| Nitrogen  | 0.01-0.015 |
| Tantalum  | 0.05-0.10  |

Molybdenum may be present in quantities less than 0.01% up to 0.50%, and preferentially between 0.1% to 0.2%, if thick sections of the alloys are desired, inasmuch as the thickness of the material is known to be a critical factor in lowering the impact strength of such alloys, which effect this additional element will counteract.

The melting of the alloys of the invention does not require special equipment or procedure, but conforms to normal practice such as, for example, open hearth, arc furnace or melting in an induction furnace. The heats thus produced can then be hot worked and normalized and further treated by tempering at various temperatures if desired.

TABLE I  
Charpy keyhole impact test (ft.-lb.) at —183° and —196° C.

|           | Percent<br>Ta<br>Added | Percent<br>Cb<br>Added | Normalized<br>900° C. |         | Normalized 900° C.       |         |                           |         |                          |         |                          |         |
|-----------|------------------------|------------------------|-----------------------|---------|--------------------------|---------|---------------------------|---------|--------------------------|---------|--------------------------|---------|
|           |                        |                        |                       |         | Temp. 600° C.—<br>1 Hour |         | Temp. 600° C.—<br>5 Hours |         | Temp. 500° C.—<br>1 Hour |         | Temp. 550° C.—<br>1 Hour |         |
|           |                        |                        | 183° C.               | 196° C. | 183° C.                  | 196° C. | 183° C.                   | 196° C. | 183° C.                  | 196° C. | 183° C.                  | 196° C. |
|           |                        |                        |                       |         |                          |         |                           |         |                          |         |                          |         |
| 2% Nickel | 0.10                   | —                      | 39.5                  | —       | 50.0                     | —       | 3.5                       | —       | —                        | —       | —                        | —       |
|           | 0.05                   | 0.05                   | 14.3                  | —       | 29.5                     | —       | 25.8                      | —       | —                        | —       | —                        | —       |
|           | 0.10                   | —                      | 13.6                  | 18.0    | 19.5                     | 21.3    | 33.5                      | 10.8    | 38.0                     | 28.5    | 41.0                     | 35.8    |
|           | 0.10                   | 0.10                   | 41.0                  | 30.0    | 26.5                     | 37.0    | 24.7                      | 5.5     | —                        | —       | —                        | —       |
|           | 0.10                   | —                      | 28.5                  | 28.0    | 34.0                     | 30.8    | 29.0                      | 3.5     | 32.0                     | 21.0    | 32.5                     | 33.8    |
|           | 0.05                   | 0.05                   | 36.5                  | 20.8    | 24.6                     | 5.5     | 29.3                      | 4.0     | —                        | —       | —                        | —       |
| 3% Nickel | 0.05                   | 0.05                   | 28.0                  | 23.5    | 33.7                     | 3.5     | 14.6                      | 16.5    | —                        | —       | —                        | —       |
|           | 0.10                   | 0.03                   | 22.3                  | 23.0    | 27.0                     | 10.8    | 27.0                      | 17.5    | —                        | —       | —                        | —       |
|           | 0.10                   | 0.03                   | 34.3                  | 33.3    | 34.8                     | 19.0    | 29.0                      | 30.3    | —                        | —       | —                        | —       |
|           | 0.25                   | —                      | —                     | 20.0    | 33.0                     | —       | —                         | 12.0    | —                        | —       | —                        | —       |
|           | 0.20                   | 0.05                   | 39.5                  | 32.5    | 35.8                     | 10.8    | 4.5                       | 8.5     | —                        | —       | —                        | —       |

It is the principal object of this invention, therefore, to provide a relatively inexpensive low alloy ferritic steel suitable for use in applications where very low temperatures are normally encountered, and which will have low transition temperatures. Another object is the provision

Referring to the attached table of impact test results, Table I, samples of similar composition were heat treated in several ways to indicate that heat treatment is not critical, and that high impact values are readily reproducible over a large number of heats in both normalized

and stress-relieved conditions. The typical nominal composition of each steel sample was:

|           | Percent |
|-----------|---------|
| Carbon    | 0.03    |
| Manganese | 0.30    |
| Silicon   | 0.20    |
| Chromium  | 0.80    |
| Copper    | 0.50    |
| Aluminum  | 0.15    |
| Nitrogen  | 0.013   |

A further indication of the effects produced by tantalum addition in lowering the transition temperature of low alloy chromium-copper-nickel steels is indicated by the data of Table II. The composition of the samples which do not contain tantalum is similar in every other respect to that of the chromium-copper-nickel steels containing 3% nickel given on Table I; the impact tests results represent an average of seven tests from four heats at a  $-183^{\circ}\text{C}$ .

The notch toughness figures for the tantalum-bearing samples are representative of 20 to 24 tests from a total of 12 heats. In nearly all cases the mean value of toughness under various heat treatments exceeds the minimum 15 foot pound criterion for low temperature application.

TABLE II

Charpy keyhole impact tests, ft.-lb.

|                                 | Normalized<br>900 °C. | Normalized<br>900 °C.,<br>Tempered<br>600 °C.—<br>1 Hour | Normalized<br>900 °C.,<br>Tempered<br>600 °C.—<br>5 Hours |
|---------------------------------|-----------------------|----------------------------------------------------------|-----------------------------------------------------------|
| Notch toughness, No Ta added... | 4.7                   | 22.3                                                     | 8.9                                                       |
| Notch toughness, Ta added.....  | 25.7                  | 30.6                                                     | 23.6                                                      |

In addition to the higher impact values obtained by the tantalum-containing alloys, the data in Table II also demonstrate that the alloys which do not contain tantalum are substantially affected by the difference in heat treatment, whereas proportionately similar results are obtained by the alloy of this invention under the different treatments.

The normalizing treatment as practiced in the present invention consists of heating the steel to above the critical temperature but not so high as to produce material grain growth and subsequently cooling at a relatively rapid rate or in some cases, in a liquid coolant. The steel is cooled substantially to room temperature prior to heating for tempering.

The exact mechanism whereby the tantalum addition lowers the transition temperature of these alloys is not known, but it is believed that this element produces a grain refinement by forming finely dispersed carbides within the grain structure and by retarding carbide solution and reprecipitation during tempering of the low alloy steel.

Columbium can be effectively added in combination with tantalum up to similar percentages as long as the total of the two elements does not exceed 0.25%. While the composition as hitherto disclosed provides excellent low temperature properties where the finished alloy bars do not exceed 1 $\frac{1}{4}$  inches in thickness, it has been found that the addition of 0.1% to 0.30% molybdenum increases the toughness of the alloy in slower-cooling, heavier sections.

By the present invention cast or wrought steel articles are produced which may be hot worked and subsequently welded, normalized, or normalized and tempered, and

which are well-suited for use in the fabrication of articles that are required to withstand severe mechanical stress at low temperatures. Their toughness upon prolonged exposure to these temperatures recommends their employment where dependable operation is essential.

What is claimed is:

1. An alloy containing about 0.02% to 0.15% carbon; 0.20% to 1.20% manganese; 0.05% to 0.60% silicon; 0.20% to 1.20% copper; 0.25% to 1.50% chromium; 1% to 5% of nickel; 0.03% to 0.30% aluminum; up to 0.025% nitrogen and 0.05% to 0.25% in the aggregate of tantalum and columbium, the tantalum content being at least 0.04%; up to 0.50% of molybdenum; and the remainder iron and incidental impurities.

15 2. An alloy containing about 0.02% to 0.15% carbon; 0.20% to 1.20% manganese; 0.05% to 0.60% silicon; 0.20% to 1.20% copper; 0.25% to 1.50% chromium; 1% to 5% of nickel; 0.03% to 0.30% aluminum; up to 0.025% nitrogen; 0.01% to 0.50% molybdenum and 20 0.05% to 0.25% in the aggregate of tantalum and columbium, the tantalum content being at least 0.04%; the remainder iron and incidental impurities.

3. An alloy containing about 0.02% to 0.10% carbon; 0.20% to 0.60% manganese; 0.10% to 0.35% silicon; 25 0.20% to 0.60% copper; 0.50% to 0.90% chromium; 2.00% to 3.00% nickel; 0.05% to 0.20% aluminum; 0.010% to 0.015% nitrogen; an aggregate of 0.05% to 0.10% of tantalum and columbium, the tantalum content being at least 0.04%; the remainder iron and incidental 30 impurities.

4. An alloy containing about 0.02% to 0.10% carbon; 0.20% to 0.60% manganese; 0.10% to 0.35% silicon; 0.20% to 0.60% copper; 0.50% to 0.90% chromium; 2.00% to 3.00% nickel; 0.05% to 0.20% aluminum; 0.010% to 0.015% nitrogen; 0.10% to 0.20% molybdenum; an aggregate of 0.05% to 0.10% of tantalum and columbium, the tantalum content being at least 0.04%; the remainder iron and incidental 35 impurities.

5. A welded article which in its normal use is required 40 to withstand mechanical stress at low temperatures down to about  $-196^{\circ}\text{C}$ , which article is composed of an alloy containing about 0.02% to 0.15% carbon; 0.20% to 1.20% manganese; 0.05% to 0.60% silicon; 0.20% to 1.20% copper; 0.25% to 1.50% chromium; 1.0% to 5% of nickel; 0.03% to 0.30% aluminum; up to 0.025% nitrogen and 0.05% to 0.25% in the aggregate of tantalum and columbium, the tantalum content being at least 0.04%; the remainder iron and incidental impurities.

6. A welded article which in its normal use is required 45 to withstand mechanical stress at low temperatures down to about  $-196^{\circ}\text{C}$ , which article is composed of an alloy containing about 0.02% to 0.15% carbon; 0.20% to 1.20% manganese; 0.05% to 0.60% silicon; 0.20% to 1.20% copper; 0.25% to 1.50% chromium; 1.0% to 5% of nickel; 0.03% to 0.30% aluminum; up to 0.025% nitrogen; 0.01% to 0.50% molybdenum and 50 0.05% to 0.25% in the aggregate of tantalum and columbium, the tantalum content being at least 0.04%; the remainder iron and incidental impurities.

7. A welded article which in its normal use is required 55 to withstand mechanical stress at low temperatures down to about  $-196^{\circ}\text{C}$ , which article is composed of an alloy containing about 0.02% to 0.10% carbon; 0.20% to 0.60% manganese; 0.10% to 0.35% silicon; 0.20% to 0.60% copper; 0.50% to 0.90% chromium; 2.00% to 3.00% nickel; 0.05% to 0.20% aluminum; 0.010% to 0.015% nitrogen; an aggregate of 0.05% to 0.10% of tantalum and columbium, the tantalum content being at least 60 0.04%; the remainder iron and incidental impurities.

8. A welded article which in its normal use is required 65 to withstand mechanical stress at low temperatures down to about  $-196^{\circ}\text{C}$ , which article is composed of an alloy containing about 0.02% to 0.10% carbon; 0.20% to 0.60% manganese; 0.10% to 0.35% silicon; 0.20% to

0.60% copper; 0.50% to 0.90% chromium; 2.00% to 3.00% nickel; 0.05% to 0.20% aluminum; 0.010% to 0.015% nitrogen; 0.10% to 0.20% molybdenum; an aggregate of 0.05% to 0.10% of columbium and tantalum, the tantalum content being at least 0.04%; the remainder 5 iron and incidental impurities.

## References Cited in the file of this patent

## UNITED STATES PATENTS

|           |               |               |
|-----------|---------------|---------------|
| 1,373,908 | Pacz          | Apr. 5, 1921  |
| 2,103,610 | Macormac      | Dec. 28, 1937 |
| 2,264,355 | Becket et al. | Dec. 2, 1941  |
| 2,679,454 | Offenhauer    | May 25, 1954  |